# EUROPEAN PATENT SPECIFICATION

(11) **EP 0 026 777 B1**
(45) Date of publication and mention of the grant of the patent: **26.10.1983**
(21) Application number: 80900685.1
(22) Date of filing: 03.04.1980
(51) Int. Cl.: D04H 1/44, D21H 5/26

(54) **METHOD FOR DISTRIBUTING FIBERS IN A LAYER**
VERFAHREN ZUM VERTEILEN VON FASERN IN EINER BESCHICHTUNG
PROCEDE DE DISTRIBUTION DE FIBRES DANS UNE COUCHE

(30) Priority: 05.04.1979 SE 7903028
(43) Date of publication of application: 15.04.1981
(73) Proprietor: OLSSON, Mats Anders, 161 39 Bromma (SE)
(72) Inventor: OLSSON, Mats Anders, 161 39 Bromma (SE)
(74) Representative: Ström, Tore
(86) International application number: SE8000098
(87) International publication number: WO8002165

## Description

The invention relates to a method for distributing fibers in a layer by exposing the fibers to a sound field.

It is previously known to treat fibers by exposing them to a sound field.

GB-A-1 092 052 describes a method of quilting fusible fibers by treating such fibers with an ultrasonic beam, the fibers being interconnected at the contact areas by a fusing action caused by the ultrasonic beam. The ultrasonic beam is emitted from a head which is pressed against the fibers.

DE-Al-2 715 747 relates to the distribution of a fiber layer by exposing the layer to ultrasonic vibration between opposite surfaces of two rigid elements which are pressed against each other.

The object of the invention is to provide a method of the art referred to above for distributing a filting fiber in a simple, cheap and rapid manner.

According to the invention, the distribution of the fibers is achieved by exposing the layer to a low-frequency air-borne sound field.

In order to illustrate the invention this will be described in more detail below, reference being made to the accompanying drawing, which shows a diagrammatic vertical cross-sectional view of an apparatus for practising the method.

The fibers 1 are laid down onto an air permeable support 2 which is arranged in front of a sound emitter 4 located in a resonator 3. In the present case the resonator 3 comprises a Helm- holtz resonator and the sound emitter 4 comprises an electric loud speaker of the diaphragm type, which is mounted in a wall of the resonator. The layer of fibers is exposed to low-frequency air-borne sound from the sound emitter 4, and by the exposure to sound the fiber layer is fluidized and spreads uniformly over the support a is indicated by a dash line 5.

If the fibers 1 are of such character that they can be entangled with each other, or if the fibers during the fluidization are sprayed with an adhesive, there will be obtained in this way a bound fiber mat of uniform thickness.

The exposure of the fiber layer to sound can also take place from the upper side of the layer.

If varying thickness of the layer is desired so that a definite profile is imparted to the layer as indicated by a dash and dot line 6, an accumulation of the fibers at one or more places as desired can be obtained by controlling the propagation of the sound field such that different portions of the fiber layer are exposed to sound fields of different strengths.

## Claims

1. Method for distributing fibers (1) in a layer by exposing the fibers to a sound field, characterized in that the fiber layer (1) is exposed to a low-frequency air-borne sound field.

2. Method according to claim 1, characterized in that the sound field is emitted from a resonator (3).

3. Method according to claim 1 or 2, characterized in that the fiber layer (1) is exposed to the sound field from below on an air permeable support (2).

4. Method according to any of claims 1 to 3, characterized in that the propagation of the sound field is controlled to actuate different portions of the fiber layer (1) with sound fields of different strengths.

5. Method according to any of claims 1 to 4 characterized in that the fiber layer (1) is sprayed with an adhesive when being exposed to the sound field.

## Patentansprüche

1. Verfahren zum Verteilen von Fasern (1) in einer Schicht durch Einwirkung eines Schallfeldes auf die Fasern, dadurch gekennzeichnet, dass die Faserschicht (1) einem niedrigfrequenten, luftübertragenen Schallfeld ausgesetzt wird.

2. Verfahren nach Anspruch 1, dadurch gekennzeichnet, dass das Schallfeld von einem Resonator (3) abgegeben wird.

3. Verfahren nach Anspruch 1 oder 2, dadurch gekennzeichnet, dass die Faserschicht (1) auf einem luftdurchlässigen Träger (2) von unten her dem Schallfeld ausgesetzt wird.

4. Verfahren nach einem der Ansprüche 1 bis 3, dadurch gekennzeichnet, dass die Ausbreitung des Schallfeldes gesteuert wird, um verschiedene Abschnitte der Faserschicht (1) Schallfeldern verschiedener Stärke auszusetzen.

5. Verfahren nach einem der Ansprüche 1 bis 4, dadurch gekennzeichnet, dass die Faserschicht (1) mit einem Klebstoff besprüht wird, während es dem Schallfeld ausgesetzt ist.

## Revendications

1. Procédé pour répartir des fibres (1) selon une couche en exposant les fibres à un champ acoustique, caractérisé en ce que la couche de fibres (1) est exposé à un champ acoustique pneumatique de basse fréquence.

2. Procédé selon la revendication 1, caractérisé en ce que le champ acoustique est émis à partir d'un résonateur (3).

3. Procédé selon la revendication 1 ou 2, caractérisé en ce que la couche de fibres (1) est exposée au champ acoustique à partir du bas sur un support (2) perméable à l'air.

4. Procédé selon l'une quelconque des revendications 1 à 3, caractérisé en ce que la propagation du champ acoustique est commandée afin de soumettre différentes parties de la couche de fibres (1) à des champs acoustiques de forces différentes.

5. Procédé selon l'une quelconque des revendications 1 à 4, caractérisé en ce qu'on arrose la couche de fibres (1) avec un adhésif lorsque celle-ci est exposée au champ acoustique.
